

# United States Patent [19]

Tsuji et al.

[11] 3,820,999

[45] June 28, 1974

[54] IMAGE-RECEIVING ELEMENT FOR USE IN  
PHOTOGRAPHIC SILVER HALIDE  
DIFFUSION TRANSFER PROCESS

[75] Inventors: Nobuo Tsuji; Takushi Miyazako;  
Kinji Ohkubo; Kazunobu Kato, all  
of Kanagawa, Japan

[73] Assignee: Fuji Photo Film Co., Ltd.,  
Kanagawa, Japan

[22] Filed: Oct. 27, 1971

[21] Appl. No.: 193,183

[30] Foreign Application Priority Data

Oct. 27, 1970 Japan ..... 45-94880

[52] U.S. Cl. ..... 96/76 R, 96/83

[51] Int. Cl. ..... G03c 1/48

[58] Field of Search ..... 96/115 P, 29, 83, 76;  
260/78

[56] References Cited

UNITED STATES PATENTS

|           |         |       |       |          |
|-----------|---------|-------|-------|----------|
| 2,698,237 | 12/1954 | Land  | ..... | 96/29    |
| 2,759,913 | 8/1956  | Hulse | ..... | 260/89.7 |
| 2,823,122 | 2/1958  | Land  | ..... | 96/29    |

3,573,922 4/1971 Rust ..... 96/115 P

OTHER PUBLICATIONS

Polymer, Vol. 11, 1970, pp. 88-110.

Primary Examiner—Ronald H. Smith

Assistant Examiner—John L. Goodrow

Attorney, Agent, or Firm—Sughrue, Rothwell, Mion,  
Zinn & Macpeak

[57] ABSTRACT

An image-receiving element for use in silver halide diffusion transfer processes, which element comprises a support having coated thereon a diffusion transfer image-receiving layer comprising a colloidal silicon dioxide containing silver-precipitating nuclei dispersed therein, said image receiving layer being overcoated with a layer containing therein poly-addition products derived from a bisacrylamide and a diamine compound, which bisacrylamide is represented by the following general formula



wherein R is a divalent hydrocarbon group having not more than 10 carbon atoms. The overcoating layer serves as a stripping layer of improved properties.

11 Claims, No Drawings

**IMAGE-RECEIVING ELEMENT FOR USE IN  
PHOTOGRAPHIC SILVER HALID DIFFUSION  
TRANSFER PROCESS**

**BACKGROUND OF THE INVENTION**

1. Field of the Invention

This invention relates to an image-receiving element for use in photographic silver salt diffusion transfer processes.

2. Description of the Prior Art

In hitherto known diffusion transfer photographic processes there are used light-sensitive photographic materials comprising a support having coated thereon a dispersion of fine particles of a light-sensitive silver salt, such as a silver halide in a hydrophilic binder such as gelatin. The light-sensitive layer thereof was exposed to light image-wisely and then contacted with a processing composition containing therein a developing agent to affect development of the exposed layer. At this point, the exposed silver halide in the light-sensitive layer is reduced (developed) to metallic silver.

Concurrently therewith, or subsequently thereto, the light-sensitive element is processed with a silver-complex forming agent, whereby a water-soluble silver complex is formed by reaction of the unexposed silver halide with the silver-complex forming agent. When, concurrently therewith, an image-receiving element having an image receiving layer containing therein a substance dispersed in a hydrophilic binder, which substance serves as a catalyst for reduction of the above-described water-soluble silver complex (said substance therefore comprising silver-precipitating nuclei or development nuclei), is brought into intimate surface contact with the aforementioned light-sensitive negative layer, the silver complex formed in the light-sensitive layer is, at least in part, transported to the image-receiving layer by diffusion. It is then reduced to silver by the effect of the development nuclei contained therein, thereby forming a positive image having a pattern corresponding to the original.

This process and the materials used therein are disclosed in detail in "Chimie et Physique Photographiques" by P. Glafkides, 3rd Ed., published by Publications Photo-Cinema Paul Montel (1967), pages 469 to 471.

In order to obtain the desired print, the image-receiving element must be dissociated or stripped from the light-sensitive element. A coating film, usually called a stripping layer, is usually provided on the image-receiving layer to facilitate the dissociation or stripping and to prevent a film of the diffusion transfer processing composition from attaching itself to and remaining on the surface of the processed image-receiving layer. When the dissociation or stripping is unsatisfactory and/or the processing composition remains thereon, the image-surface of the image-receiving element is tainted and the quality of the image is remarkably lowered. Furthermore, in the absence of such a stripping layer on the image-receiving element, the silver images formed on the image-receiving element frequently undergo deterioration upon storage and/or the highlight areas thereof yellow.

As materials for the aforementioned stripping layer, there have been previously employed, for example,

gum arabic, hydroxyethyl cellulose, methyl cellulose, polyvinyl alcohol, polymethacrylate, resins and sodium alginate.

Although the above-mentioned materials are effective to stop processing composition remaining on the surface of the positive print, and to protect the surface of the image-receiving sheet from being scratched during handling, they often present disadvantages in that the transferred image assumes a metallic luster and/or the maximum density of the positive image is lowered.

**SUMMARY OF THE INVENTION**

The present invention thus relates to an image-receiving element useful for silver halide diffusion transfer photographic processes, which element comprises a support having coated thereon a diffusion transfer image-receiving layer mainly comprising colloidal silicon dioxide containing silver precipitating nuclei dispersed therein, said image-receiving layer being overcoated with a layer containing poly-addition products derived from a bisacrylamide and a diamine compound which bisacrylamide may be represented by the following general formula:



wherein R is a divalent hydrocarbon group defined hereinafter.

An object of the present invention is to provide the aforementioned image-receiving material which yields a positive print free from deteriorated silver images or yellowed areas even in its highlight areas.

Another object of the present invention is to provide the aforementioned image-receiving material which has a surface protected from being scratched on handling.

**DETAILED DESCRIPTION OF THE INVENTION**

The condensation products which characterize the present invention may be prepared by the poly-addition of bisacrylamide to diamine compound. The representative polycondensation condition is provided in "Polymer" vo. 11, page 88 (1970).

One of the starting materials, bisacrylamide, may be represented by the following general formula



wherein R stands for a divalent hydrocarbon group such as



n being a number from 1 to 10,



The other starting material, the diamine compound may be, for example, ethylene diamine, 1,3-propanediamine, hexamethylene diamine, piperidine, xylylene diamine, phenylene diamine. According to our study, the condensation products wherein, above all, ethylene diamine, 1,3-propane diamine or piperidine are used have been found to be most suitable for accomplishing the afore-mentioned objects of the present invention. Furthermore, the lower the number of carbon atoms in the R group in the bisacrylamide, the bet-

ter the results which are obtained. The intrinsic viscosity [n] of the addition-polymerization products, which reflects the polymerization degree thereof, preferably ranges from 0.005 to 0.5, particularly from 0.01 to 0.1. In this specification, intrinsic viscosity is measured in water at 30° C.

Specific examples of such poly-addition products will be illustrated by the following.

(Compound 1)

The poly-addition product of methylene bisacrylamide and ethylene diamine having an intrinsic viscosity  $n_{H_2O}^{30^\circ} C$  of 0.085.

(Compound 2)

The poly-addition product of methylene bisacrylamide and piperadine having an intrinsic viscosity  $n_{H_2O}^{30^\circ} C$  of 0.090.

(Compound 3)

The poly-addition product of ethylene bisacrylamide and piperidine having an intrinsic viscosity  $n_{H_2O}^{30^\circ} C$  of 0.065.

(Compound 4)

The poly-addition products of methylene bisacrylamide and 1,3-propane diamine having an intrinsic viscosity  $n_{H_2O}^{30^\circ} C$  of 0.070.

These poly-addition products are all soluble in water or alcohols, so that they can be applied, in the form of a solution in water, alcohol or a mixture of water and alcohol, to the surface of an image-receiving element.

The coating weight of the products is in the range of from about 0.1 to about 2.0 g/m<sup>2</sup>, preferably from 0.3 to 1.0 g/m<sup>2</sup>. If the coverage is much less than the recited range, the effect of preventing attachment of the processing composition tends to be lessened while if the coverage exceeds the range, diffusion transfer tends to be inhibited.

As the support for use in the image-receiving element according to the present invention, there may be employed any suitable material used as such supports by the prior art, for example, films or sheets of film-

forming resins such as polyethylene terephthalate, cellulose triacetate, polycarbonate, polyvinyl chloride or polyethylene, baryta-coated paper, resin-coated papers, glass plates, metal plates, plates made of earthenware or like materials.

As silver precipitating nuclei useful in the present invention, there may be preferably employed the normally water-insoluble sulfides, or selenides of Cd, Pt, Zn, Cu, Co, Ni, Fe, Sn, Au, Ag, etc., or colloidal heavy

or noble metal, such as of Au, Ag, Pt, Pd, Hg, etc., having an average size of less than 10 microns, it being desirable that the silver precipitating nuclei in the image-receiving element be of high activity. In particular, image-receiving elements utilizing highly active silver precipitating nuclei can be preferentially used as high speed diffusion transfer photographic materials. U.S. Pat. No. 2,698,237 describes a method for preparing such highly active silver precipitating nuclei, wherein a water-soluble metal salt and water-soluble sulfide are admixed in particulate silicon dioxide, thereby forming a precipitate of the resulting water-insoluble metal sulfide. Any other hitherto known techniques for forming such silver precipitating nuclei can be applied to the present invention.

25 The operable ratio of the silver precipitating nuclei: colloidal silicon dioxide in the layer is within 1:5 to 1:1,000 by weight, preferably 1:50 to 1:200.

The colloidal silicon dioxide which has incorporated therein the silver-precipitating nuclei and also serves as 30 a binder is also known as anhydrous silicic acid, and per se is an acidic substance. When it is dispersed in water, it is in part hydrated to form silicic acid. The pKa and pKa<sub>2</sub> of silicic acid are 9.8 and 12.16 at 30° C, respectively. It is desirable that the silicon dioxide used in the present invention be in the form of particles which are as fine as possible such as less than 1 micron. Examples of silicon dioxides suitable for use in the present invention and commercially available are listed in the following table. In the last column of the table are shown pH

| Maker                                      | Trade Name  | Form                      | pH       |
|--------------------------------------------|-------------|---------------------------|----------|
| Monsanto Chemical Co.                      | Santocel 54 | 4% aqueous dispersion     | 3.8      |
|                                            | do. C       | do.                       | 3.8      |
|                                            | do. L       | do.                       | 4.0      |
|                                            | do. 62      | do.                       | 3.8      |
|                                            | do. FRC     | do.                       | 3.8      |
| Nippon Aerosil K.K.                        | Aerosil 130 | 4% aqueous dispersion     | 3.6-4.3  |
|                                            | do. 200     | do.                       | 3.6-4.3  |
|                                            | do. 300     | do.                       | 3.6-4.3  |
|                                            | do. 0       | do.                       | 3.6-4.3  |
|                                            | do. 380     | do.                       | 3.6-4.3  |
|                                            | do. MOX80   | do.                       | 3.6-4.2  |
|                                            | do. COK84   | do.                       | 3.8-4.6  |
|                                            | do. MOK170  | do.                       | 3.6-4.2  |
|                                            |             |                           |          |
| W.R. Grace & Co. Davison Chemical Division | Syloid 308  | 5% aqueous dispersion     | 2.4      |
|                                            | do. 404     | do.                       | 7.0      |
|                                            | do. AL-1    | do.                       | 3.8      |
|                                            | do. 65      | do.                       | 3.8      |
|                                            | do. 978     | do.                       | 2.4      |
|                                            | do. 161     | do.                       | 7.0      |
|                                            | do. 162     | do.                       | 7.0      |
|                                            | do. 244     | do.                       | 7.0      |
|                                            | do. 75      | do.                       | 7.0      |
|                                            |             |                           |          |
| E.I. du Pont de Nemours & Co.              | Ludox HS-40 | 40.1% aqueous dispersion  | 9.6      |
|                                            | do. HS-30   | 30.1%                     | 9.8      |
|                                            | do. LS      | 30.1%                     | 8.3      |
|                                            | do. AS      | 30.1%                     | 9.4      |
|                                            | do. AM      | 30%                       | 9.1      |
|                                            | do. SM      | 30%                       | 9.9      |
| Nissan chemical Industries, Ltd.           | Snowtex 20  | 20-21% aqueous dispersion | 9.5-10.0 |
|                                            | do. 30      | 30-31%                    | 9.5-10.5 |
|                                            | do. 40      | 40-41%                    | 9.5-10.5 |
|                                            | do. C       | 20-21%                    | 8.5-9.0  |
|                                            | do. N       | do.                       | 8.0-9.5  |
|                                            | do. O       | do.                       | 3.0-4.0  |
|                                            |             |                           |          |

values of aqueous dispersions of the respective silicon dioxides. These values are all reported by their makers. As previously stated, an aqueous dispersion of silicon dioxide is in itself, acidic. However, to prevent gelation, silicon dioxide is often commercially available in the form of alkaline aqueous dispersions having a pH of 3.5 to 12, but the preferable range of pH is from 6 to 9.

Image-receiving elements according to the present invention may be prepared by dispersing the aforementioned silver-precipitating nuclei into such colloidal silicon dioxides, applying the dispersion onto a support followed by drying and providing on the resulting layer the stripping layer containing the aforementioned poly-addition products, the effective and preferred combined thickness of their layers being within 0.1 to 20 microns, more preferably 0.5 to 5 microns. To the poly-addition product layer may also be incorporated surface active agents such as saponin, and to silicon dioxide layer may be incorporated such a surface active agent, a toning agent such as triphenyl-5-mercapto tetrazole or benzimidazole, a reducing agent such as phenidone, polyethanolamine, ethanol amine, glycerine, hydroquinone etc.

The thus obtained image-receiving element can accomplish the aforementioned objects and is very useful as a diffusion transfer photographic material.

The present invention will be further explained in detail with particular reference to the following Comparison Examples and Examples.

#### COMPARISON EXAMPLE 1

An aqueous dispersion of silver-precipitating nuclei was prepared by mixing the following ingredients:

|                                                   |        |
|---------------------------------------------------|--------|
| 5% by weight, aqueous solution of "Santocel 54"   |        |
| (trade name, silicon dioxide manufactured by      |        |
| Monsanto Chemical Co.)                            | 250 cc |
| 2% by weight, aqueous solution of lead acetate    |        |
| (trihydrate)                                      | 1.5 cc |
| 3% by weight, aqueous solution of cadmium acetate |        |
| (dihydrate)                                       | 2.3 cc |
| 5% by weight, aqueous solution of zinc nitrate    |        |
| (pentahydrate)                                    | 5.0 cc |
| 3% by weight, aqueous solution of sodium sulfide  |        |
| (monohydrate)                                     | 1.0 cc |
| 6% by weight, aqueous solution of saponin         | 5.0 cc |

The dispersion was applied to the surface of a baryta-coated paper at a coverage of 20 cc/m<sup>2</sup>.

The image-receiving element thus obtained was then brought into intimate contact with imagewise exposed "Neopan SSS sheet film" (trade name, highly sensitive photographic negative material using a silver iodobromide emulsion provided by Fuji Photo Film Co., Ltd.) in a manner such that the image-receiving layer was surface contacted with the emulsion sheet, between which was spread a viscous diffusion transfer photographic processing composition having the following composition:

|                                        |       |   |
|----------------------------------------|-------|---|
| Water                                  | 1,860 | g |
| Sodium salt of carboxymethyl cellulose | 117   | g |
| Sodium sulfite (anhydrous)             | 78    | g |
| Sodium hydroxide                       | 74.6  | g |
| Sodium thiosulfate (crystalline)       | 14.5  | g |
| Citric acid                            | 38.5  | g |
| Hydroquinone                           | 52    | g |

The negative element and the image-receiving element were kept in contact with each other for a period

of 15 seconds to effect the diffusion transfer of the images, after which the image-receiving element was stripped off the negative element. The resulting positive print on the image-receiving element was covered with a film of the processing composition and tainted brown.

#### Comparison Example 2

A solution having the following composition:

|                                      |     |    |
|--------------------------------------|-----|----|
| Gum arabic (Iwaki Seiyaku Co., Ltd.) | 2.0 | g  |
| Distilled water                      | 100 | cc |
| 6% aqueous solution of saponin       | 2.0 | cc |

was applied onto the coating of the image-receiving element prepared in Comparison Example 1 at a coverage of 20 cc/m<sup>2</sup>, and then dried. The image-receiving element thus obtained was then processed in the same manner as in Comparison Example 1.

After 15 seconds of processing, the image-receiving element was separated from the negative element and it was found that the processing composition film adhered only to the negative element, but not to the image-receiving element. However, the maximum density of the resulting positive images was 0.80 in terms of reflection density. Furthermore, the transferred images in the areas of high density assumed a metallic luster.

#### EXAMPLE 1

On top of the coating of the image-receiving element prepared in Comparison Example 1 there was coated an aqueous solution having the following composition:

|                                                                                                           |        |
|-----------------------------------------------------------------------------------------------------------|--------|
| Poly-addition product of methylene bisacrylamide and ethylenediamine                                      |        |
| (intrinsic viscosity $n_{H_2O}^{30^\circ C} = 0.085$ ,<br>see below with regard to the synthesis thereof) | 2.0 g  |
| 6% aqueous solution of saponin                                                                            | 100 cc |

1 N aqueous caustic soda solution to adjust the pH to 7.

The coverage was 20 cc/m<sup>2</sup>. The element was then dried, thereby forming a stripping layer.

Synthesis of the above-described poly-addition product

Into a 2,000 cc round bottom flask equipped with a stirrer and cooling tube were charged 154 g of methylene bisacrylamide and a solution of 60 g of ethylenediamine in 800 cc of formamide. These compounds were reacted with each other by stirring them at a temperature of from 120° to 140° C for a period of 5 hours. After the reaction was completed the reaction products were precipitated in an excess of acetone and the resulting solids dried in vacuo. The products weighed 195 g. and the yield was 91.2%. The mean number molecular weight was 350 and the intrinsic viscosity  $n_{H_2O}^{30^\circ C} = 0.085$ .

The image-receiving element obtained as described above was then diffusion transfer processed in the same manner as Comparison Example 1, thereby obtaining a positive print without any processing composition remaining thereon.

The maximum density of the transferred positive image was 1.50 in terms of reflection density, and no metallic luster was observed even in the areas of high density.

## EXAMPLE 2

On top of the coating of the image-receiving element prepared in Comparison Example 1, there was coated an aqueous solution having the following composition:

|                                                                                                                        |        |
|------------------------------------------------------------------------------------------------------------------------|--------|
| Poly-addition product of methylene bisacrylamide and piperazine (intrinsic viscosity $n_{H_2O}^{30^\circ} c = 0.090$ ) | 2.5 g  |
| Distilled water                                                                                                        | 100 cc |
| 6% aqueous solution of saponin                                                                                         | 2.0cc  |

1 N aqueous caustic soda solution was added thereto to adjust the pH to 7.0 at a coverage of 20 cc/m<sup>2</sup>. The element was then dried, thereby forming a stripping layer.

The image-receiving element thus obtained was then diffusion transfer processed in the same manner as Comparison Example 1, thereby obtaining a positive print without any processing composition film remaining thereon.

The maximum density of the transferred positive images was 1.20 in terms of reflection density, and no metallic luster was observed even in areas of high density.

## EXAMPLE 3

On top of the coating of the image-receiving element prepared in Comparison Example 1, there was coated an aqueous solution having the following composition:

|                                                                                                                                |        |
|--------------------------------------------------------------------------------------------------------------------------------|--------|
| Poly-addition product of methylene bisacrylamide and 1,3-propanediamine (intrinsic viscosity $n_{H_2O}^{30^\circ} c = 0.070$ ) | 20 g   |
| Distilled water                                                                                                                | 100 cc |
| 6% aqueous solution of saponin                                                                                                 | 2.0 cc |

1 N aqueous caustic soda solution to adjust the pH to 7.0 at a coverage of 20 cc/m<sup>2</sup>. The element was then dried, thereby forming a stripping layer.

The image-receiving element thus obtained was then diffusion transfer processed in the same manner as Comparison Example 1, thereby obtaining a positive print without any processing composition film remaining thereon.

The maximum density of the transferred positive image was 1.00 in terms of reflection density, and no metallic luster was observed, even in the areas of high density.

As is evident from the above-described examples, the image-receiving element coated with the compounds of the present invention are remarkably superior to the hitherto known elements coated with other compounds, in that developing composition films are neither attached nor left on the positive element of the invention, and the maximum density of the transferred images is high.

Furthermore, in an image-receiving element having coated thereon the compounds of the invention any scratching during handling is avoided, and no processing composition film remains on the positive surface, so that any deterioration of the resulting silver images or brown-tainting by oxidation products contained in the processing composition will not occur.

Although the invention has been described in considerable detail with reference to certain embodiments

thereof, it will be understood that variations and modifications can be effected without departing from the spirit and scope of the invention as described hereinabove and defined in the appended claims.

5. What we claim is:

1. In an image-receiving element for use in silver halide diffusion transfer photographic processes which comprises a support having coated thereon a diffusion image-receiving layer comprising a colloidal silicon dioxide containing silver-precipitating nuclei dispersed therein, the improvement which comprises said image-receiving layer being overcoated with a layer containing poly-addition products derived from a bisacrylamide represented by the following general formula:



wherein R is a divalent hydrocarbon group selected from the group consisting of  $-\text{CH}_2-\text{CH}(\text{CH}_3)-$ ,  $-(\text{CH}_2)_n-$  where n is an integer of 1 to 10,



and a diamine compound selected from the group consisting of ethylene diamine, 1,3-propane diamine, hexamethylene diamine, piperazine, xylene diamine and phenylene diamine, said silver precipitating nuclei being a member selected from the group consisting of water-insoluble metal sulfides, metal selenides, colloidal heavy metals and colloidal noble metals.

2. The image-receiving element as claimed in claim 1 wherein said bisacrylamide is methylene bisacrylamide and said diamine compound is ethylene diamine.

3. The image-receiving element as claimed in claim 1 wherein said bisacrylamide is methylene bisacrylamide and said diamine compound is piperazine.

4. The image-receiving element as claimed in claim 1 wherein said bisacrylamide is ethylene bisacrylamide and said diamine compound is ethylene diamine.

45 5. The image-receiving element as claimed in claim 1 wherein said bisacrylamide is methylene bisacrylamide and said diamine compound is 1,3-propanediamine.

6. The image-receiving element as claimed in claim 1 wherein said poly-addition products have an intrinsic viscosity  $n_{H_2O}^{30^\circ} c$  of from 0.005 to 0.5.

7. The image-receiving element as claimed in claim 1 wherein said image-receiving layer is overcoated with a poly-addition products in the form of a solution in a member selected from the group consisting of water, an alcohol or a mixture of water and an alcohol.

8. The image-receiving element as claimed in claim 1, wherein said image-receiving layer is overcoated with the poly-addition products at a coverage of from 0.1 to 2.0 g./m<sup>2</sup>.

9. The image-receiving element as claimed in claim 1 wherein the weight ratio of said silver precipitating nuclei: said colloidal silicon dioxide varies from 1:5 to 1:1000.

65 10. The image-receiving element as claimed in claim 1 wherein said colloidal silicon dioxide has a particle size of less than 1 micron.

11. The image-receiving element as claimed in claim 1 wherein said silver precipitating nuclei are selected from the group consisting of water insoluble sulfides and selenides of cadmium, platinum, zinc, copper, cobalt, nickel, iron, tin, gold and silver and colloidal

heavy and noble metals selected from the group consisting of gold, silver, platinum, palladium and mercury, said silver precipitating nuclei having an average particle size of less than 10 microns.

5

\* \* \* \* \*

10

15

20

25

30

35

40

45

50

55

60

65

UNITED STATES PATENT OFFICE  
CERTIFICATE OF CORRECTION

Patent No. 3,820,999 Dated June 28, 1974

Inventor(s) Nobuo TSUJI et al

It is certified that error appears in the above-identified patent and that said Letters Patent are hereby corrected as shown below:

IN THE CLAIMS:

Column 8, claim 1, line 25 - change the right-hand structural formula to the following:



Signed and sealed this 11th day of March 1975.

(SEAL)

Attest:

RUTH C. MASON  
Attesting Officer

C. MARSHALL DANN  
Commissioner of Patents  
and Trademarks